

## PROCESS FOR THE PRODUCTION OF PATTERNED TONE-ON-TONE EFFECTS ON A THERMOPLASTIC MATERIAL

Fred Fortress and Fred Best, Charlotte, N.C., assignors to Celanese Corporation of America, New York, N.Y., a corporation of Delaware

No Drawing. Filed Feb. 20, 1957, Ser. No. 641,265

6 Claims. (Cl. 8—14)

This invention relates to the production of patterned effects in fabrics of cellulose acetate of high acetyl content.

It is an object of this invention to provide a fabric of cellulose acetate of high acetyl content having a novel patterned effect.

Another object of this invention is the production of fabrics of novel patterned effect in which all parts of the fabric are dyed in the same color and in which the fabric is substantially smooth.

Other objects of this invention will be apparent from the following detailed description and claims. In this description and claims all proportions are by weight unless otherwise indicated.

In accordance with one aspect of this invention, a fabric of yarns of cellulose acetate of high acetyl content is embossed in a pattern by pressing a heated patterned embossing surface against said fabric. The embossed fabric is then dyed and, preferably, heat-treated. During dyeing and heat-treating the embossed effect on the fabric substantially disappears; that is, the fabric returns to substantially its original smooth texture, with the previously embossed portions in substantially the same plane as the unembossed portions. However, the resulting smooth fabric has a definite two-tone, or tone-on-tone, appearance showing, by differences in shade, the pattern originally applied by embossing.

The cellulose acetate of high acetyl content referred to above has an acetyl value of at least 59%, preferably at least 61%, calculated as combined acetic acid. For best results, the cellulose acetate, before it is subjected to the treatment of this invention, is in that crystalline condition corresponding to a safe ironing temperature of below about 200° C. It is desirable that the fabric be composed entirely of fibers of the cellulose acetate of high acetyl content. However, fabrics composed of blends of fibers of cellulose acetate of high acetyl content with non-thermoplastic fibers such as cotton, linen, wool, and rayon may also be used, although the results are not as good as when an unblended cellulose acetate of high acetyl content is used alone. Best results have been obtained with woven fabrics but the process of this invention may be applied to knitted, knotted or non-woven fabrics as well.

As stated, the embossing surface should be heated. Excellent results have been obtained when the embossing surface is at a temperature of about 200° C. to 220° C. In one convenient method the fabric is passed continuously into contact with a heated patterned metal embossing roll, being pressed resiliently against the raised portions of the embossing roll by means of a suitable smooth, resilient-surfaced pressure roll.

The embossing is carried out in such a manner that only portions of the fabric which are in contact with the raised portions of the heated embossing surface are subjected to the elevated temperature of said embossing surface, to achieve spot heat treatment, the other parts

of the fabric being out of contact, or not pressed firmly into contact, with said heated embossing surface and therefore being at a lower temperature. The extent of embossing may be varied as desired. An embossing roll in which the raised surfaces are  $\frac{1}{16}$  inch above the remainder of the roll surface has been found very suitable for use with fabrics having thicknesses of about  $\frac{1}{200}$  to  $\frac{1}{40}$  inch. The embossing treatment should not be so severe as to cause fusion of adjacent fibers and loss of the fibrous character of the fabric or to damage said fabric, as by severing the fibers thereof.

After the embossing operation the fabric is dyed with a disperse cellulose acetate dyestuff, preferably in a heated aqueous dyebath containing a dispersing agent and, if desired, a dyeing assistant. The dyestuff and dyeing assistant used, and the dyeing procedures employed, may be any of those described in the copending application of V. S. Salvin et al., Serial No. 472,758, filed December 2, 1954. During dyeing the embossed fabric loses at least a portion of its embossed texture and becomes flatter. The dyed fabric shows a patterned tone-on-tone effect, the portions of the fabric which had been in contact with the raised portions of the heated embossing surface having a lighter appearance than the other portions of the fabric.

After dyeing the fabric is heat-treated. The effect of this heat-treatment is to raise the safe-ironing point of the fabric, as well as to improve its resistance to glazing, its resistance to shrinkage on pressing with moist steam, and its wash fastness. The heat-treatment also increases the crystallinity and crystalline order index of the cellulose acetate of high acetyl content.

In the heat-treatment step the conditions disclosed in the aforesaid copending application of Salvin et al. may be employed. This heat-treatment results in a further flattening of the fabric so that substantially none of its original embossed texture remains.

It is desirable to apply a finish to the fabric before heat-treatment. One very suitable finish is the mixture comprising an aqueous dispersion of a silicone and colloidal silica, described in Fortress et al. application Serial No. 529,073, filed August 17, 1955.

The tone-on-tone effect produced in accordance with this invention is highly resistant to washing and cleaning and the patterned fabrics of this invention have substantially the same hand, feel and drape as fabrics which have not undergone any embossing treatment. The same tone-on-tone effect is not produced when the same process is carried out except that the embossing is done after the dyeing, but before the heat treatment.

While this invention finds its greatest utility for fabrics of cellulose acetate of high acetyl value, the same treatment may also be used for fabrics of polyesters of high melting point, such as polyethylene terephthalate, to produce similar effects.

The following examples are given to illustrate this invention further.

*Example I*

60 A woven fabric composed of fibers of cellulose acetate of acetyl value 61.5%, calculated as combined acetic acid, and having a safe ironing temperature of below 200° C. is passed into contact with a copper embossing roll having its surface formed in a small repeated four-leaf-clover pattern. The embossing roll is maintained at a temperature of 210° C. and the fabric is pressed against the embossing roll by means of a smooth metal roll having a uniform paper cover. The time of contact between embossing roll and fabric is 0.04 second. 65 The embossed fabric, in which the slightly raised outlines of the pattern are evident, is then dyed a medium blue shade in an aqueous dyebath containing 8% based

on the weight of the fabric, of Eastman Blue GLF (1,8 dihydroxy-5-nitro-4 - alpha - hydroxyethyl phenyl amino anthraquinone) and 1% based on the weight of the fabric, of "Igepon T Gel" (sodium tauryl sulfate) at a liquor ratio (ratio of weight of dyebath to weight of fabric) of 8:1, for four hours at a temperature of 95° C. After washing, the dyed fabric is heat treated by means of a radiant heater at a fabric temperature of 220° C. for 12 seconds. The resulting fabric is substantially smooth and flat and has an overall two-tone four-leaf-clover pattern. The treatment does not change the hand or drape of the fabric.

*Example II*

Example I is repeated except that a dyeing assistant (5 grams per liter of "Emkala" plus 3 grams per liter of "Emkatex") is substituted for the "Igepon T." The effect is the same as in Example I except that the shade of the fabric is darker.

*Example III*

Example I is repeated except that the fabric is scoured after the embossing treatment and before dyeing. Also, just before the heat-treatment the fabric is finished with a silicone-silica finish as described in Fortess et al. application Serial No. 529,073. The flat, heat-treated fabric retains its tone-on-tone patterned appearance even after boiling for one hour.

*Example IV*

Example III is repeated, except that the similar dye, Interchemical Blue GSF, is used. The results are substantially the same.

It is to be understood that the foregoing detailed description is given merely by way of illustration and that many variations may be made therein without departing from the spirit of our invention.

Having described our invention what we desire to secure by Letters Patent is:

1. Process for the production of patterned tone-on-tone effect fabrics which comprises embossing, with a heated surface at a temperature of about 200° to 220° C., a fabric of cellulose acetate of acetyl value at least 59%, calculated as combined acetic acid, and then dyeing said fabric with a disperse cellulose acetate dyestuff and substantially removing the embossed texture of the fabric, to produce an unembossed flat fabric having a tone-on-tone pattern.
2. Process as set forth in claim 1, and comprising the step of heat-treating said fabric after dyeing to raise the safe ironing temperature of said fabric to at least 220° C., from an initial value, before embossing, of not over 200° C.
3. Process as set forth in claim 1 in which said acetyl values is at least 61%.
4. Process as set forth in claim 1 in which said dyeing is carried out in a heated aqueous dyebath containing said dyestuff.
5. A fabric produced in accordance with claim 1.
6. A fabric produced in accordance with claim 3.

References Cited in the file of this patent

UNITED STATES PATENTS

|           |                    |               |
|-----------|--------------------|---------------|
| 1,557,461 | Lauten -----       | Oct. 13, 1925 |
| 2,750,250 | Lindenstruth ----- | June 12, 1956 |

FOREIGN PATENTS

|         |                     |               |
|---------|---------------------|---------------|
| 598,716 | Great Britain ----- | Feb. 25, 1948 |
|---------|---------------------|---------------|

OTHER REFERENCES

35 "The Technical Bulletin," pub. by the Du Pont Co., September 1955, pp. 115-120.